# EUROPEAN PATENT SPECIFICATION

(11) **EP 3 717 144 B1**
(45) Date of publication and mention of the grant of the patent: **24.01.2024**
(21) Application number: 18804345.9
(22) Date of filing: 26.11.2018
(51) Int. Cl.: B21J 5/00, B22D 18/02, B22D 18/04, B22D 27/11, B22D 33/02

(54) **METHOD FOR CASTING AND FORGING OBJECTS MADE OF BRASS, BRONZE, ALUMINUM ALLOYS, LIGHT ALLOYS AND THE LIKE**
VERFAHREN ZUM GIESSEN UND SCHMIEDEN VON GEGENSTÄNDEN AUS MESSING, BRONZE, ALUMINIUMLEGIERUNGEN, LEICHTMETALLEGIERUNGEN UND DERGLEICHEN
PROCÉDÉ PERMETTANT DE COULER ET DE FORGER DES OBJETS EN LAITON, EN BRONZE, EN ALLIAGES D'ALUMINIUM, EN ALLIAGES LÉGERS ET ANALOGUES

(30) Priority: 27.11.2017 IT 201700135597
(43) Date of publication of application: 07.10.2020
(73) Proprietor: Euromac Srl, 36035 Marano Vicentino (IT)
(72) Inventor: FRULLA, Claudio, 20084 Lacchiarella (IT)
(74) Representative: Modiano, Micaela Nadia
(86) International application number: PCT/EP2018/082517
(87) International publication number: WO 2019/101989

(56) References cited:
- WO-A1-2017/115259
- US-A- 3 866 666
- US-B1- 7 216 692

## Description

The present invention relates to a method for casting and forging objects made of brass, bronze, aluminum alloys, light alloys and the like. A method according to the preamble of claim 1 is e.g. known from WO2017/115259 A1.

More particularly, the invention relates to a method for providing objects at low pressure and forged in the semisolid state.

As is known, in the production of objects with small and medium dimensions, there are problems in the quality of the product, which must not have impurities of gas or air, must have the lowest possible cycle time, and must also have high mechanical characteristics.

In the background art an apparatus is known which is provided with a lower die and an upper die which form an area for the containment of a dosed quantity of liquid metal that arrives from a duct arranged in communication with a furnace and arrives from below.

In this technical solution, the upper die is provided with a flow control element which acts on a connecting port of the liquid metal inlet duct and a compaction punch, which forms a portion of the upper impression of the die.

The die is then filled by overflow with the liquid metal, but with the drawback of not knowing exactly the quantity of metal that is required to complete the part.

Furthermore, metal dosage might be incorrect, since in the initial step the die is not filled completely but the liquid metal reaches the level of the overflow line, thus achieving total filling of the die only after the closure of the port for connection to the liquid metal inlet duct and the descent of the compaction punch which causes the liquid metal to rise to complete the casting cavity.

The solution proposed above is susceptible of improvements. Furthermore, the solution described above allows to process one part at a time, with accordingly considerable process times.

The aim of the present invention is to provide a method for casting objects made of brass, bronze, aluminum, light alloys in general and the like, that allow to obtain cast parts that are free from gas or air impurities in the shortest possible cycle time.

Within this aim, an object of the present invention is to provide a method for casting objects made of brass, bronze, aluminum, light alloys and the like that can be used even if a core made of sand or the like has been inserted in the casting cavity.

Another object of the present invention is to provide a method for casting objects made of brass, bronze, aluminum, light alloys and the like that allowed to provide process steps simultaneously on multiple parts being processed.

A further object of the present invention is to provide a method that is highly reliable, relatively simple to provide and at competitive costs.

This aim, as well as these and other objects which will become better apparent hereinafter, are achieved by a method as defined in independent claim 1.

Further characteristics and advantages of the invention will become better apparent from the description of a preferred but not exclusive embodiment of the method according to the invention, illustrated by way of non-limiting example in the accompanying drawings, wherein:
Figure 1 is a perspective view of the apparatus suitable for carrying out the method according to the present invention;
Figure 2 is a partially sectional front elevation view of the apparatus suitable for carrying out the method according to the invention;
Figure 3 is another partially sectional front elevation view of the apparatus suitable for carrying out the method according to the invention;
Figure 4 is a top plan view of the apparatus suitable for carrying out the method according to the present invention;
Figure 5 is a partial and partially sectional front elevation view of a first step of the casting method according to the present invention;
Figure 6 is a partial and partially sectional front elevation view of a second step of the casting method according to the present invention;
Figure 7 is a partial and partially sectional front elevation view of a third step of the casting method according to the present invention;
Figure 8 is a partial and partially sectional front elevation view of a fourth step of the casting method according to the present invention;
Figure 9 is a sectional front elevation view of a detail of the apparatus suitable for carrying out the method according to the invention.

With reference to the figures, the apparatus suitable for carrying out the method according to the invention is described first and then the method for using it.

In all the figures, identical reference numerals correspond to identical elements.

The casting apparatus, designated generally by the reference numeral 1, comprises a turntable 2 on which at least three dies 3 are mounted which are adapted to be arranged at a matching number of processing stations.

In particular, the turntable 2 mounts three dies 3 and a fourth die, the purpose of which will be clarified better hereinafter.

The apparatus thus provides for a transfer of each die 3 from one station to another by rotation of the turntable 2.

The first station 5 is a casting station below which there is a pressurized furnace 15 for introducing the liquid metal 16 in the cavity of the die 3 that is present at the station 5.

The second station is a station in which the upper die part is opened, carrying with it the cast part until the part is extracted.

The second station is designated by the reference numeral 6.

The third station, designated by the reference numeral 7, is a station for the cooling and lubrication of the die. The open die is transferred by means of the turntable 2 to a fourth station 8, where a metal or sand or ceramic core, designated in the figures by the reference numeral 10, is inserted in the casting cavity.

Once the die is closed, the rotation of the turntable 2 is actuated for the transfer of the closed die back to the first station 5.

While in the first station 5 liquid metal is introduced and its forging and solidification occur, at the same time in the station 6 the extraction of the part previously cast in the first station 5 is performed and, again simultaneously, in the third station 7 cooling of the die with corresponding lubrication is performed and in the fourth station 8 the core is inserted in the open die, previously cooled and lubricated in the third station 7, and the closure of the die 3 is actuated, again simultaneously, at the first, second and third stations.

Essentially, therefore, the method according to the invention provides for a simultaneous processing of the apparatus at the four stations, with the dies 3 being moved from one station to the other by rotation of the turntable 2.

In this manner, the method according to the invention allows to perform simultaneous processing on multiple stations, enormously speeding up the process times.

As is known, components of a core made of sand and the like can be obtained only with foundry processes in which a maximum pressure of 2 kg/cm² is applied to the liquid metal. It is instead not possible to provide components with a core made of sand or the like with foundry processes in which high pressure is applied to the liquid metal, for example pressure die casting.

With the method according to the invention the filling of the liquid metal in the casting cavity is performed at low pressure (approximately 2 kg/cm²) and, when the casting cavity is filled with the liquid metal 16 and with the core made of sand or the like 10 surrounded by the liquid metal, high pressure is applied to the metal undergoing solidification, with values that can reach even for example 1200 kg/cm².

This is possible by using the fourth processing station 8.

In detail, in the first station 5 the die 3 comprises a lower die part 3a and an upper die part 3b, which are closed.

Furthermore, the station 5 comprises a forging punch 11, within which a flow control element 12 slides. The forging punch 11 in turn slides within a guiding bushing 13.

In the first station 5, therefore, when the die 3 is closed, the forging punch 11 is inserted in the guiding bushing 13 that is arranged at the upper part 3b of the die. The forging punch 11 is moved in its descent by a slider, which therefore performs a vertical descent so as to insert the forging punch 11 in the guiding bushing 13, as mentioned. The slider continues its stroke in order to apply a closing force between the upper die part 3b and the lower die part 3a.

Then the furnace 15 for feeding the liquid metal 16 that is located below the first station 5 is pressurized.

In the figures, the cast part is designated by the reference numeral 20.

The casting steps described above are illustrated in Figures 5 to 8.

When the die 3 passes with the cast part 20 at the second station 6, the extraction of the part cast is performed in the station 5 and transferred together with the die 3 to the station 6 by means of the turntable 2, which performs a rotation of 90° if the apparatus comprises four stations, or a rotation of 120° if the apparatus comprises only three stations.

The cooling and lubrication of the die is performed, as mentioned, at the third station 7. Cooling is entrusted to a plurality of nozzles 15 and 16 which respectively cool the upper die part 3b and the lower die part 3a.

All the operations in the various stations are performed simultaneously.

The fourth station 8 is the one in which the core made of metal or sand or ceramic is inserted in the die 3, which was previously cooled and lubricated at the third station 7 and transferred to the fourth station 8 by means of a further rotation of the turntable 2.

The fourth station 8 is obviously used only for the objects to be cast that have in cross-section a cavity in which the presence of a core 10 is required.

When the core 10 is inserted at the fourth station 8, a cylinder located on the turntable 2 is actuated and closes the die 3 with the core 10 inserted therein.

When the die is closed, the rotation of the turntable 2 is actuated again to transfer the closed die 3 to the first station 5.

While in the first station the introduction of the liquid metal 16 and the corresponding forging are performed, at the same time in the second station 6 the extraction of the part cast previously is performed and in the third station 7, again simultaneously, the cooling of the die 3 and the corresponding lubrication is performed, and in the fourth station 8 the core 10 is inserted in the open die 3, which arrives from the third station 6.

In practice it has been found that the casting method according to the invention achieves the intended aim and objects, since it allows to perform simultaneous processes on three or more dies 3, at a matching number of processing stations, thus speeding up the casting process.

The method thus conceived furthermore allows to provide components with cores made of sand and the like.

The method thus conceived is susceptible of numerous modifications and variations, all of which are within the scope of the appended claims.

All the details may furthermore be replaced with other technically equivalent elements.

In practice, the materials used, as well as the contingent shapes and dimensions, may be any according to the requirements and the state of the art.

Where technical features mentioned in any claim are followed by reference signs, those reference signs have been included for the sole purpose of increasing the intelligibility of the claims and accordingly such reference signs do not have any limiting effect on the interpretation of each element identified by way of example by such reference signs.

## Claims

1. A method for casting and forging objects made of brass, bronze, aluminum alloys, light alloys and the like, comprising the steps of:
at a first station (5), performing the forging of a part (20) by means of a die (3) composed of an upper die part (3b) and a lower die part (3a);
transferring said die (3) to a second station (6) for the extraction of said part (20);
transferring said die (3) to a third station (7) for the cooling and lubrication of said die;
said steps being performed simultaneously with each other,the method further comprising a step of inserting a core (10) within said die (3), said step of inserting a core within said die following said step of cooling and lubricating said die (3) and preceding said forging step, **characterized in that** in said forging step liquid metal (16) is filled in the casting cavity at low pressure, of approximately 2 kg/cm², and, when said casting cavity has been filled with metal and with the core (10) surrounded by the liquid metal (16), high pressure, of even 1200 kg/ cm², is applied to the metal that is in the solidification step.

2. The method according to claim 1, **characterized in that** the transfer of said dies (3) from one station to another is performed by means of a turntable (2) on which said dies (3) are supported.

## Patentansprüche

1. Ein Verfahren zum Gießen und Schmieden von Gegenständen aus Messing, Bronze, Aluminiumlegierungen, Leichtmetalllegierungen und dergleichen, das folgende Schritte umfasst:
an einer ersten Station (5), das Schmieden eines Teils (20) mit Hilfe einer Form (3), die aus einem oberen Formabschnitt (3b) und einem unteren Formabschnitt (3a) besteht;
das Transportieren der Form (3) zu einer zweiten Station (6) zur Extraktion des Teils (20);
das Transportieren der Form (3) zu einer dritten Station (7) zum Kühlen und Schmieren der Form;
wobei die Schritte gleichzeitig durchgeführt werden; wobei das Verfahren weiter einen Schritt des Einsetzens eines Kerns (10) in die Form (3) umfasst, wobei der Schritt des Einsetzens eines Kerns in die Form dem Schritt des Kühlens und Schmierens der Form (3) folgt und dem Schmiedeschritt vorausgeht; **dadurch gekennzeichnet, dass** in dem Schmiedeschritt Flüssigmetall (16) mit niedrigem Druck von ungefähr 2 kg/cm² in den Gusshohlraum eingefüllt wird und wenn der Gusshohlraum mit Metall und mit dem vom Flüssigmetall (16) umgebenen Kern (10) gefüllt wurde, Hochdruck von sogar 1200 kg/cm² auf das Metall ausgeübt wirkt, das sich im Erstarrungsschritt befindet.

2. Das Verfahren gemäß Anspruch 1, **dadurch gekennzeichnet, dass** der Transport der Formen (3) von einer Station zur anderen mit Hilfe eines Drehtischs (2) durchgeführt wird, auf welchem die Formen (3) gelagert sind.

## Revendications

1. Procédé pour couler et forger des objets en laiton, en bronze, en alliages d'aluminium, en alliages légers et analogues, comprenant les étapes consistant à :
au niveau d'un premier poste (5), effectuer le forgeage d'une partie (20) au moyen d'une matrice (3) composée d'une partie de matrice supérieure (3b) et d'une partie de matrice inférieure (3a) ;
transférer ladite matrice (3) vers un deuxième poste (6) pour l'extraction de ladite partie (20) ;
transférer ladite matrice (3) vers un troisième poste (7) pour le refroidissement et la lubrification de ladite matrice ;
lesdites étapes étant effectuées simultanément les unes avec les autres, le procédé comprenant en outre une étape d'insertion d'un noyau (10) à l'intérieur de ladite matrice (3), ladite étape d'insertion d'un noyau à l'intérieur de ladite matrice suivant ladite étape de refroidissement et de lubrification de ladite matrice (3) et précédant ladite étape de forgeage, **caractérisé en ce que**, lors de ladite étape de forgeage, du métal liquide (16) est rempli dans la cavité de coulée à basse pression, d'approximativement 2 kg/cm², et, lorsque ladite cavité de coulée a été remplie de métal et du noyau (10) entouré par le métal liquide (16), une haute pression, même de 1 200 kg/cm², est appliquée au métal qui est dans l'étape de solidification.

2. Procédé selon la revendication 1, **caractérisé en ce que** le transfert desdites matrices (3) d'un poste à un autre est effectué au moyen d'un plateau tournant (2) sur lequel lesdites matrices (3) sont supportées.
